

May 9, 1961

M. HUMENIK, JR., ET AL

2,983,034

METAL GRAPHITE COMPACTS

Filed Nov. 25, 1959



M. HUMENIK, JR.  
R. L. VAN ALSTEN  
INVENTORS

BY

J. R. Faulkner  
G. H. Oster  
ATTORNEYS

1

2,983,034

## METAL GRAPHITE COMPACTS

Michael Humenik, Jr., Inkster, and Roy L. Van Alsten, Detroit, Mich., assignors to Ford Motor Company, Dearborn, Mich., a corporation of Delaware

Filed Nov. 25, 1959, Ser. No. 855,321

14 Claims. (Cl. 29—182.5)

This invention relates to the powdered metal art and is more specifically concerned with powdered metal compacts in which unusually large percentages of graphite or diamond are bonded into strong and useful objects by relatively small percentages of metal. Despite the well-known weakness and brittleness of graphite and diamond and their resistance to ordinary sintering procedures it has been possible to produce objects having very acceptable physical properties. This invention is related to application Serial No. 610,956, filed September 20, 1956, now forfeited; application Serial No. 708,685, filed January 13, 1958, now abandoned; applications Serial Nos. 708,815, 708,816 and 708,817, all filed January 14, 1958, now abandoned; and application Serial No. 733,873, filed May 8, 1958, now abandoned.

Successful sintered compacts have been fabricated in which the metal component has been selected from the group of metals consisting of iron, cobalt, nickel, copper, silver and aluminum. These metals have been employed to bond together large amounts of either graphite or diamond.

The unusual physical properties of these metal graphite or metal diamond compacts are obtained by sintering the green compact at a temperature sufficiently high to insure that essentially all of the metal content of the compact is in the liquid phase. The exact temperature of the sintering operation will depend on the melting point of the metal phase. Since all of the metal phase is in the liquidus state during sintering it is necessary to take certain precautions to prevent the molten metal from sweating out of the compact and collecting as globules on the surface of the compact.

The figure of drawing which is a section through a globule of metal resting on a graphite stool has been presented to enable a better understanding of this invention.

In the drawing a graphite stool has been denominated 10. A globule of molten metal has been denominated 11. A tangent 12 has been drawn to globule 11 where globule 11 intersects graphite stool 10. Angle A is the angle included between tangent 12 and the upper surface of the graphite stool as measured through the globule. The inventors have discovered that as long as the angle A is substantially not in excess of ninety degrees, metal of the constitution of that in globule 11 may be incorporated in a graphite compact and sintered above the melting point of the globule without substantial loss of metal due to sweating.

Mathematically angle A may be defined as follows: Cosine A is equal to the difference between the surface energy of the graphite and the solid liquid interfacial energy, this difference being divided by the surface tension of the liquid phase. Or, otherwise expressed,

$$\cosine A = \frac{E_s - E_{sl}}{E_l}$$

2

where  $E_s$  is the surface energy of the solid,  $E_{sl}$  is the solid liquid interfacial energy and  $E_l$  is the surface tension of the liquid.

This invention is predicated upon the fact that a graphite-metal compact, or a diamond-metal compact can be sintered at a temperature above the melting point of the metal without any sweating provided there is present in the compact as an alloying ingredient at least one of the following group of metals:

10

Calcium  
Barium  
Strontium  
Magnesium

The amounts of calcium, barium, strontium, and magnesium to be added to the graphite-metal compact or diamond-metal compact are not critical. Economic factors will usually limit the addition of these elements to the smallest amount which will produce effective results. However, within reason larger amounts will do no harm. Because of its cheapness and ready availability, calcium in the form of calcium silicide is preferred for the practice of this invention. As little as 0.1 percent calcium silicide has been found to be effective in preventing sweating of iron from compacts. Approximately 5 percent calcium silicide appears to produce optimum results. However, this invention has been executed employing as the additional material barium in the form of barium silicide, and magnesium in the form of magnesium ferro silicon. The calcium silicide composition was approximately 33 percent calcium, remainder silicon. The barium silicide was approximately 45 percent barium, remainder silicon. The magnesium ferro silicon had a composition of about 11 percent magnesium, 39 percent iron and the remainder silicon.

To illustrate this invention the following specific examples are given.

Iron graphite compacts were prepared from iron powder and graphite powder which had been separately ground to pass a 140 mesh screen and then ball milled together in benzene for four hours to insure proper mixing. The mixture was cold pressed in a hardened steel die using pressures of 50,000 to 100,000 pounds per square inch. The compacts were sintered in a vacuum of from 100 to 200 microns and in ambients of hydrogen, helium and argon. The temperature of sintering was 2400° F. and the time was sixty minutes.

The following compacts were fabricated from graphite powder and a mixture consisting of 5 percent by weight calcium silicide and 95 percent by weight iron powder. Any size iron powder from 60 to 325 mesh is suitable. The compositions given in the table below are in volume percentages.

| Iron, calcium silicide | Graphite | Transverse<br>rupture<br>strength,<br>p.s.i. | Resistivity<br>ohm in— |
|------------------------|----------|----------------------------------------------|------------------------|
| 10                     | 90       | 4,180                                        | 0.000152               |
| 20                     | 80       | 13,700                                       | 0.000064               |
| 30                     | 70       | 21,100                                       | 0.000045               |
| 40                     | 60       | 28,600                                       | 0.000036               |
| 50                     | 50       | 38,800                                       | 0.000031               |

The following compacts were fabricated from graphite powder and a mixture consisting of 5 percent by weight barium silicide and 95 percent by weight iron powder. The compositions given in the table below are 70 in volume percentages.

| Iron, barium silicide | Graphite | Transverse<br>rupture<br>strength,<br>p.s.i. | Resistivity<br>ohm in— |
|-----------------------|----------|----------------------------------------------|------------------------|
| 10.....               | 90       | 2,080                                        | 0.000248               |
| 30.....               | 70       | 6,660                                        | 0.000075               |
| 50.....               | 50       | 18,600                                       | 0.000045               |

The following compacts were fabricated from graphite powder and a mixture of 15 percent magnesium ferro silicon and 85 percent iron powder. The compositions given in the table below are in volume percentages.

| Iron, ferro silicon | Graphite | Transverse<br>rupture<br>strength,<br>p.s.i. | Resistivity<br>ohm in— |
|---------------------|----------|----------------------------------------------|------------------------|
| 10.....             | 90       | 6,540                                        | 0.000104               |
| 30.....             | 70       | 17,500                                       | 0.000061               |
| 50.....             | 50       | 41,500                                       | 0.000056               |

A further series of compacts were prepared containing 5.0 percent calcium silicide and the following properties were obtained.

| Metal volume, percent               | 10     | 20     | 30     | 40     | 50     |
|-------------------------------------|--------|--------|--------|--------|--------|
| Transverse rupture strength, p.s.i. | 5,500  | 14,500 | 21,000 | 28,250 | 40,000 |
| Tensile strength, p.s.i.            | 6,500  | 10,900 | 14,800 | 19,500 |        |
| Compressive strength, p.s.i.        | 11,400 | 14,400 | 25,500 | 51,300 |        |
| Elongation, percent                 | 0      | 0.5    | 1.0    | 2.0    |        |
| Porosity, percent                   | 21.7   | 20.8   | 22.9   | 19.5   | 18.8   |

The above compacts were sintered for one hour at a temperature of 2300° F. in vacuum.

Cobalt graphite compacts were prepared from cobalt powder and graphite powder which had been separately ground to pass a 325 mesh screen and then ball milled together in benzene for four hours to insure proper mixing. The mixture was cold pressed in a hardened steel die using pressures of 50,000 to 100,000 pounds per square inch. The compacts were sintered in a vacuum of from 100 to 200 microns and in ambients of hydrogen, helium and argon. The temperature of sintering was 2500° F. and the time was sixty minutes.

The following compacts were fabricated from graphite powder and a mixture consisting of 5 percent by weight calcium silicide and 95 percent by weight cobalt powder. A cobalt powder of 325 mesh is suitable. The compositions given in the following table are in volume percentages.

| Cobalt, calcium silicide | Graphite | Transverse<br>rupture<br>strength,<br>p.s.i. | Resistivity<br>ohm in— |
|--------------------------|----------|----------------------------------------------|------------------------|
| 10.....                  | 90       | 6,120                                        | .000132                |
| 30.....                  | 70       | 16,000                                       | .000066                |
| 50.....                  | 50       | 28,400                                       | .000043                |

The following compacts were fabricated from graphite powder and a mixture consisting of 5 percent by weight barium silicide and 95 percent by weight cobalt powder. The compositions given in the table below are in volume percentages.

| Cobalt, barium silicide | Graphite | Transverse<br>rupture<br>strength,<br>p.s.i. | Resistivity<br>ohm in— |
|-------------------------|----------|----------------------------------------------|------------------------|
| 10.....                 | 90       | 1,640                                        | .000365                |
| 30.....                 | 70       | 3,920                                        | .000146                |
| 50.....                 | 50       | 6,850                                        | .000078                |

The following compacts were fabricated from graphite powder and a mixture of 15 percent magnesium ferro

silicon and 85 percent cobalt powder. The compositions given in the table below are in volume percentages.

| 5       | Cobalt, ferro silicon | Graphite | Transverse<br>rupture<br>strength,<br>p.s.i. | Resistivity<br>ohm in— |
|---------|-----------------------|----------|----------------------------------------------|------------------------|
| 10..... | 90                    | 5,900    | .000130                                      |                        |
| 30..... | 70                    | 19,100   | .000064                                      |                        |
| 50..... | 50                    | 30,600   | .000056                                      |                        |

Copper graphite compacts were prepared from copper powder and graphite powder which had been separately ground to pass a 200 mesh screen and then ball milled together in benzene for four hours to insure proper mixing. The mixture was cold pressed in a hardened steel die using pressures of 50,000 to 100,000 pounds per square inch. The compacts were sintered in a vacuum of from 100 to 200 microns and in ambient of hydrogen, helium and argon. The temperature of sintering was 2000° F. and the time was sixty minutes.

The following compacts were fabricated from graphite powder and a mixture consisting of 5 percent by weight calcium silicide and 95 percent by weight copper powder.

25 A copper powder of 200 mesh is suitable. The compositions given in the table below are in volume percentages.

| 30      | Copper, calcium silicide | Graphite | Transverse<br>rupture<br>strength,<br>p.s.i. | Resistivity<br>ohm in— |
|---------|--------------------------|----------|----------------------------------------------|------------------------|
| 10..... | 90                       | 2,110    | .000748                                      |                        |
| 30..... | 70                       | 2,830    | .000233                                      |                        |
| 50..... | 50                       | 4,490    | .000070                                      |                        |

The following compacts were fabricated from graphite powder and a mixture consisting of 5 percent by weight barium silicide and 95 percent by weight copper powder. The compositions given in the table below are in volume percentages.

| 40      | Copper, barium silicide | Graphite | Transverse<br>rupture<br>strength,<br>p.s.i. | Resistivity<br>ohm in— |
|---------|-------------------------|----------|----------------------------------------------|------------------------|
| 10..... | 90                      | 1,710    | .000518                                      |                        |
| 30..... | 70                      | 3,230    | .000152                                      |                        |
| 50..... | 50                      | 4,540    | .000069                                      |                        |

The following compacts were fabricated from graphite powder and a mixture of 15 percent magnesium ferro silicon and 85 percent copper powder. The compositions given in the table below are in volume percentages.

| 55      | Copper, ferro silicon | Graphite | Transverse<br>rupture<br>strength,<br>p.s.i. | Resistivity<br>ohm in— |
|---------|-----------------------|----------|----------------------------------------------|------------------------|
| 10..... | 90                    | 1,710    | .000513                                      |                        |
| 30..... | 70                    | 2,540    | .000159                                      |                        |
| 50..... | 50                    | 5,640    | .000085                                      |                        |

The following compacts were fabricated from graphite powder and a mixture of 15 percent of copper magnesium and 85 percent copper powder. The compositions given in the following table are in volume percentages.

| 60      | Copper, copper magnesium | Graphite | Transverse<br>rupture<br>strength,<br>p.s.i. | Resistivity<br>ohm in— |
|---------|--------------------------|----------|----------------------------------------------|------------------------|
| 10..... | 90                       | 1,090    | .000410                                      |                        |
| 30..... | 70                       | 1,240    | .000092                                      |                        |
| 50..... | 50                       | 2,630    | .000078                                      |                        |

Nickel graphite compacts were prepared from nickel powder and graphite powder which had been separately

ground to pass a 140 mesh screen and then ball milled together in benzene for four hours to insure proper mixing. The mixture was cold pressed in a hardened steel die using pressures of 50,000 to 100,000 pounds per square inch. The compacts were sintered in a vacuum of from 100 to 200 microns and in ambients of hydrogen, helium and argon. The temperature of sintering was 2500° F. and the time was sixty minutes.

The following compacts were fabricated from graphite powder and a mixture consisting of 5 percent by weight calcium silicide and 95 percent by weight nickel powder. A nickel powder of 325 mesh is suitable. The compositions given in the table below are in volume percentages.

| Nickel, calcium silicide | Graphite | Transverse<br>rupture<br>strength,<br>p.s.i. | Resistivity<br>ohm in— |
|--------------------------|----------|----------------------------------------------|------------------------|
| 10.....                  | 90       | 4,015                                        | .000200                |
| 30.....                  | 70       | 6,150                                        | .000113                |
| 50.....                  | 50       | 10,150                                       | .000060                |

The following compacts were fabricated from graphite powder and a mixture consisting of 5 percent by weight barium silicide and 95 percent by weight nickel powder. The compositions given in the table below are in volume percentages.

| Nickel, barium silicide | Graphite | Transverse<br>rupture<br>strength,<br>p.s.i. | Resistivity<br>ohm in— |
|-------------------------|----------|----------------------------------------------|------------------------|
| 10.....                 | 90       | 2,250                                        | .000333                |
| 30.....                 | 70       | 3,980                                        | .000143                |
| 50.....                 | 50       | 6,490                                        | .000057                |

The following compacts were fabricated from graphite powder and a mixture of 15 percent magnesium ferro silicon and 85 percent nickel powder. The compositions given in the table below are in volume percentages.

| Nickel, ferro silicon | Graphite | Transverse<br>rupture<br>strength,<br>p.s.i. | Resistivity<br>ohm in— |
|-----------------------|----------|----------------------------------------------|------------------------|
| 10.....               | 90       | 4,730                                        | .000198                |
| 30.....               | 70       | 11,000                                       | .000100                |
| 50.....               | 50       | 18,400                                       | .000100                |

The following compacts were fabricated from graphite powder and a mixture of 20 percent nickel magnesium and 80 percent nickel. The compositions given in the following table are in volume percentages. The composition of the nickel magnesium is nickel 84 percent and magnesium 16 percent.

| Nickel Magnesium | Graphite | Transverse<br>rupture<br>strength,<br>p.s.i. | Resistivity<br>ohm in— |
|------------------|----------|----------------------------------------------|------------------------|
| 10.....          | 90       | 2,850                                        | .000214                |
| 30.....          | 70       | 2,400                                        | .000081                |
| 50.....          | 50       | 8,290                                        | .000042                |

The following compacts were fabricated from graphite powder and a mixture consisting of 5 percent by weight calcium silicide and 95 percent by weight silver powder. The compositions given in the table below are in volume percentages.

| Silver, calcium silicide | Graphite | Transverse<br>rupture<br>strength,<br>p.s.i. | Resistivity<br>ohm in— |
|--------------------------|----------|----------------------------------------------|------------------------|
| 30.....                  | 70       | 1,660                                        | 0.000068               |
| 50.....                  | 50       | 2,720                                        | 0.000011               |

The calcium silicide contained approximately 33 percent calcium.

The following compacts were prepared from graphite powder and a mixture consisting of 5 percent by weight barium silicide and 95 percent by weight silver powder. The compositions given in the following table are in volume percentages.

| 10      | Silver, barium silicide | Graphite | Transverse<br>rupture<br>strength,<br>p.s.i. | Resistivity<br>ohm in— |
|---------|-------------------------|----------|----------------------------------------------|------------------------|
| 30..... | 50.....                 | 70       | 1,780                                        | 0.000082               |

The barium silicide contained approximately 45 percent barium, remainder substantially all silicon.

Three aluminum graphite compacts have been fabricated. They were designated S1-17, S1-27, and S1-28. The composition of these are as follows:

|           | S1-17    | S1-27    | S1-28 |
|-----------|----------|----------|-------|
| Mg—7.24   | Cu—7.7   | Cu—3.57  |       |
| Tl—0.015  | Mg—4.94  | Mg—1.46  |       |
| Zn—3.02   | Ni—0.55  | Ni—2.04  |       |
| Al—89.725 | Mn—0.48  | Mn—0.10  |       |
|           | Tl—0.11  | F—0.10   |       |
|           | Fe—0.10  | Si—0.10  |       |
|           | Al—86.12 | Tl—0.02  |       |
|           |          | Al—92.79 |       |

The density of these alloys was calculated and these turned out to be:

|            | Gm./cc. |
|------------|---------|
| S1-17..... | 2.76    |
| S1-27..... | 3.21    |
| S1-28..... | 3.02    |

They were filed down by hand into powders to pass through a 100 mesh screen.

They were then mixed with the Acheson graphite 38 powder in 50-50 by volume proportions.

These were pressed in a hardened steel die and sintered in vacuum at 1800° F.

No sweating was observed.

Compacts of equal parts by volume of a minus 325 mesh diamond powder and a mixture of 10 percent by weight of calcium silicide powder and 90 percent by weight of copper powder were formed by pressing the pre-mixed powders in a hardened steel die at a pressure of 100,000 p.s.i. These compacts were sintered in an argon atmosphere to a temperature of 2020° F. A sound, hard sintered compact resulted with all the metallic phase being retained in the compact.

Similar results were obtained with compacts formed by pressing at 100,000 p.s.i., containing equal parts by volume of a minus 325 mesh diamond powder and a mixture composed of 10 percent by weight of calcium silicide powder and 90 percent by weight of silver powder. These compacts were sintered in an argon atmosphere at 1850° F.

We claim:

1. A sintered metal bonded composition containing as essential ingredients a substance selected from the group of substances consisting of graphite and diamond and between ten and seventy percent by volume metal selected from the group of metals consisting of iron, cobalt, nickel, copper, silver and aluminum, and a small but effective addition of at least one metal selected from the group of metals consisting of calcium, magnesium, barium and strontium, said addition being present in an amount sufficient to substantially prevent the metal content of the composition from sweating out during the sintering operation.

2. A sintered metal bonded graphite composition containing as essential ingredients graphite and between ten and seventy percent by volume metal selected from the

group of metals consisting of iron, cobalt, nickel, copper, silver and aluminum, and a small but effective addition of at least one metal selected from the group of metals consisting of calcium, magnesium, barium and strontium, said addition being present in an amount sufficient to substantially prevent the metal content of the composition from sweating out during the sintering operation.

3. A sintered metal bonded diamond composition containing as essential ingredients diamond and between ten and seventy percent by volume metal selected from the group of metals consisting of iron, cobalt, nickel, copper, silver and aluminum, and a small but effective addition of at least one metal selected from the group of metals consisting of calcium, magnesium, barium and strontium, said addition being present in an amount sufficient to substantially prevent the metal content of the composition from sweating out during the sintering operation.

4. A sintered metal bonded graphite composition containing as essential ingredients graphite and between ten and seventy percent by volume iron, and a small but effective addition of at least one metal selected from the group of metals consisting of calcium, magnesium, barium and strontium, said addition being present in an amount sufficient to substantially prevent the metal content of the composition from sweating out during the sintering operation.

5. A sintered metal bonded graphite composition containing as essential ingredients graphite and between ten and seventy percent by volume cobalt, and a small but effective addition of at least one metal selected from the group of metals consisting of calcium, magnesium, barium and strontium, said addition being present in an amount sufficient to substantially prevent the metal content of the composition from sweating out during the sintering operation.

6. A sintered metal bonded graphite composition containing as essential ingredients graphite and between ten and seventy percent by volume nickel, and a small but effective addition of at least one metal selected from the group of metals consisting of calcium, magnesium, barium and strontium, said addition being present in an amount sufficient to substantially prevent the metal content of the composition from sweating out during the sintering operation.

7. A sintered metal bonded graphite composition containing as essential ingredients graphite and between ten and seventy percent by volume copper, and a small but effective addition of at least one metal selected from the group of metals consisting of calcium, magnesium, barium and strontium, said addition being present in an amount sufficient to substantially prevent the metal content of the composition from sweating out during the sintering operation.

8. A sintered metal bonded graphite composition containing as essential ingredients graphite and between ten and seventy percent by volume aluminum, and a small but effective addition of at least one metal selected from the group of metals consisting of calcium, magnesium, barium and strontium, said addition being present in an amount sufficient to substantially prevent the metal content of the composition from sweating out during the sintering operation.

9. A sintered metal bonded diamond composition con-

taining as essential ingredients diamond and between ten and seventy percent by volume iron, and a small but effective addition of at least one metal selected from the group of metals consisting of calcium, magnesium, barium and strontium, said addition being present in an amount sufficient to substantially prevent the metal content of the composition from sweating out during the sintering operation.

10. A sintered metal bonded diamond composition containing as essential ingredients diamond and between ten and seventy percent by volume cobalt, and a small but effective addition of at least one metal selected from the group of metals consisting of calcium, magnesium, barium and strontium, said addition being present in an amount sufficient to substantially prevent the metal content of the composition from sweating out during the sintering operation.

11. A sintered metal bonded diamond composition containing as essential ingredients diamond and between ten and seventy percent by volume nickel, and a small but effective addition of at least one metal selected from the group of metals consisting of calcium, magnesium, barium and strontium, said addition being present in an amount sufficient to substantially prevent the metal content of the composition from sweating out during the sintering operation.

12. A sintered metal bonded diamond composition containing as essential ingredients diamond and between ten and seventy percent by volume copper, and a small but effective addition of at least one metal selected from the group of metals consisting of calcium, magnesium, barium and strontium, said addition being present in an amount sufficient to substantially prevent the metal content of the composition from sweating out during the sintering operation.

13. A sintered metal bonded diamond composition containing as essential ingredients diamond and between ten and seventy percent by volume aluminum, and a small but effective addition of at least one metal selected from the group of metals consisting of calcium, magnesium, barium and strontium, said addition being present in an amount sufficient to substantially prevent the metal content of the composition from sweating out during the sintering operation.

14. A sintered metal bonded graphite composition containing as essential ingredients graphite and between ten and seventy percent by volume iron, and a small but effective addition of calcium, said addition being present in an amount sufficient to substantially prevent the metal content of the composition from sweating out during the sintering operation.

55 1,053,880 Scott et al. Feb. 18, 1913

1,636,763 Boring July 26, 1927

1,775,358 Smith Sept. 9, 1930

2,191,936 Lenel Feb. 27, 1946

60 2,416,830 Heuberger Mar. 4, 1947

#### References Cited in the file of this patent

#### UNITED STATES PATENTS

|              |                            |
|--------------|----------------------------|
| 55 1,053,880 | Scott et al. Feb. 18, 1913 |
| 1,636,763    | Boring July 26, 1927       |
| 1,775,358    | Smith Sept. 9, 1930        |
| 2,191,936    | Lenel Feb. 27, 1946        |
| 60 2,416,830 | Heuberger Mar. 4, 1947     |

#### FOREIGN PATENTS

|         |                            |
|---------|----------------------------|
| 172,693 | Great Britain Dec. 1, 1921 |
| 465,936 | Great Britain May 13, 1937 |